

Dec. 27, 1966

S. FOLDES ETAL

3,294,497

COATED COLUMBIUM OR TANTALUM BASE METAL

Filed Jan. 26, 1966

2 Sheets-Sheet 1

FIG. 1.



FIG. 2.



Inventors:  
Stephen Foldes  
Moses A. Levinstein  
by *Richard J. Burgess*  
Their Attorney

Dec. 27, 1966

S. FOLDES ET AL

3,294,497

COATED COLUMBIUM OR TANTALUM BASE METAL

Filed Jan. 26, 1966

2 Sheets-Sheet 2

FIG. 3.



PRESENCE OF EUTECTIC AFTER FUSION TREATMENT

FIG. 4.

$\text{CbAl}_3 + \text{Ag-Si Alloy Eutectic}$



APPEARANCE OF EUTECTIC AFTER OXIDATION

Inventors:  
Stephen Foldes  
Moses A. Levinstein  
by *Richard H. Burgess*  
Their Attorney

## 1

3,294,497  
COATED COLUMBIUM OR TANTALUM  
BASE METAL

Stephen Foldes, San Jose, Calif., and Moses A. Levinstein, Cincinnati, Ohio, assignors to General Electric Company, a corporation of New York

Filed Jan. 26, 1966, Ser. No. 523,220  
7 Claims. (Cl. 29—194)

This application is a continuation-in-part of applicants' copending application Ser. No. 232,896, now abandoned, filed October 24, 1962.

This invention relates to an oxidation resistant article of a refractory metal or metal alloy and more particularly to an aluminide coating system on notch-sensitive refractory metals.

The oxidation resistance of a wide variety of metals and their alloys has been improved through the use of the metal aluminum as a surface coating, usually alloyed with the base metal, at least at the interface between the two. Such a coating may be referred to as an aluminum-base coating or an aluminide coating because of the formation of an aluminide of the base metal, as for example a columbium aluminide. These coatings have been applied in a variety of ways including the application of powdered material and by various molten spray and molten dip techniques, for example as shown in Patent 3,186,070, Gordon D. Oxx, patented June 1, 1965 and assigned to the same assignee as the present invention.

It is well known that various alloys of aluminum can be used to provide oxidation resistant coatings on refractory metals, particularly columbium (also known as niobium) and tantalum and alloy systems based on these metals. However, most of the coatings of this type currently known are subject to the handicaps of being quite brittle, causing serious notch embrittlement of the base metal, or both. These effects are especially harmful to the high strength alloys of columbium, many of which are inherently notch sensitive to some extent. A very brittle coating also has the disadvantage of forming a network of fine cracks which allow air to reach the substrate thereby causing contamination and resulting embrittlement of the base metal.

On the other hand, some of the compounds formed between refractory metals and aluminum are highly oxidation resistant and therefore desirable as coatings. For example, three intermetallic compounds can be prepared in the columbium-aluminum system, namely  $\text{Cb}_3\text{Al}$ ,  $\text{Cb}_2\text{Al}$ , and  $\text{CbAl}_3$ . Of the columbium aluminides  $\text{CbAl}_3$  is the most oxidation resistant as well as the most brittle phase. Corresponding phase relations exist in the tantalum-aluminum system, and the coatings herein described are equally useful on columbium or columbium-base alloys and tantalum or tantalum-base alloys.

It is an object of this invention to provide a highly oxidation resistant article of columbium or tantalum or an alloy based on one of these metals having an oxidation resistant aluminum-base coating with minimum susceptibility to crack propagation through the coating or into the base metal.

These and other objects and advantages will be recognized from the following detailed description and examples and the accompanying drawing.

Briefly stated, in one form, the present invention provides an article of a refractory metal or alloy having a first coating of silver bonded thereto of a thickness sufficient to cover the entire surface and a second coating of powder metal aluminum-base alloy bonded to said silver coating. The composite body is heat treated to fuse the coatings together and to the base metal.

In another form, the present invention provides an article of columbium or tantalum or an alloy of either,

## 2

on the surface of which has been fused an aluminide coating in the form of either  $\text{CbAl}_3$  or  $\text{TaAl}_3$ , which aluminide coating includes silver in solid solution.

In another form, the present invention provides an oxidation resistant article of columbium or tantalum or an alloy of either having an aluminide coating fused to the surface thereof, the coating being predominantly  $\text{CbAl}_3$  or  $\text{TaAl}_3$  with silver and another metal, preferably silicon, in solid solution, the coating having a silver and silicon rich portion adjacent the interface between the coating and the base metal. Upon exposure to air at elevated temperatures, an outer skin of  $\text{Al}_2\text{O}_3$  forms, and an inner layer converts from  $\text{CbAl}_3$  or  $\text{TaAl}_3$  to  $\text{Cb}_2\text{Al}$  or  $\text{Ta}_2\text{Al}$ , respectively, with silver and silicon precipitating therefrom. There is some intermixing of these layers.

In each of these embodiments of the invention, an outer coating of aluminum metal may be provided over an aluminum alloy coating.

In the drawings, FIG. 1 is a photomicrograph of a 20 coating system of the invention, and FIG. 2 is a photomicrograph of the same coating after an oxidation treatment. FIG. 3 is an electron photomicrograph at high 25 magnification illustrating the ductile eutectic formed in the region of the coating-base metal interface according to the invention. FIG. 4 is the same as FIG. 3 but after a two-hour oxidation treatment at 2500° F.

Wherever  $\text{Cb}_2\text{Al}$ ,  $\text{CbAl}_3$ ,  $\text{Ta}_2\text{Al}$  or  $\text{TaAl}_3$  are referred to in this specification, it should be understood that complex aluminides of the form  $\text{M}_2\text{Al}$  and  $\text{MAl}_3$  are meant to be included. M is representative of the base metal which can be columbium, a columbium-base alloy, tantalum, or a tantalum-base alloy. For example, in a columbium-base alloy containing 15 percent titanium, M would represent  $(\text{Cb}, \text{Ti})$  and  $\text{M}_2\text{Al}$  would be  $(\text{Cb}, \text{Ti})_2\text{Al}$ . In like manner, when other metals such as, for example, chromium, silicon or titanium are added to the aluminum alloy coating, the coating would contain the complex aluminides of columbium and some or all of the other metals present in either the coating or the base metal alloy.

Broadly stated the present invention preferably provides an article of manufacture comprising a body of a base metal selected from the group consisting of columbium, columbium-base alloys, tantalum, and tantalum-base alloys, and a protective coating integral with an exposed surface of said body to protect it against oxidation while not destroying the ductility of the base metal by greatly increased sensitivity to crack propagation, said coating being bonded together and to said base metal by diffusion and comprising: a continuous layer of a continuous phase of a monometal trialuminide having a composition in the proportion of one atom at least predominantly of the selected one of the base metals columbium and tantalum to each three atoms of aluminum, said layer containing sufficient amounts of silver in solution so that as excess of the selected one of the base metals columbium and tantalum diffuses into said layer upon exposure to elevated temperatures and an oxidizing atmosphere, a ductile eutectic containing silver, aluminum and the selected one of the base metals columbium and tantalum forms at a substantial portion of the grain boundaries of said monometal trialuminide and acts as a barrier to the propagation of cracks from said layer into said base metal.

Upon continued exposure to elevated temperatures such as at about 2500° F. for about two hours in an oxidizing atmosphere, a continuous layer of  $\text{Al}_2\text{O}_3$  forms at the exposed surface of the monometal trialuminide, thereby depleting the aluminum content of the aluminide, and the columbium or tantalum of the base metal diffuses out into the coating, causing the formation of a di-metal aluminide having a composition in the proportion of two atoms at least predominantly of the selected one of the

base metals columbium and tantalum to each atom of aluminum. This di-metal aluminide forms into a continuous layer at the interface between the base metal and the monometal trialuminide of the balance of the coating, and the layer grows in thickness with time. Ultimately, in the case of columbium and columbium-base alloys, when the  $\text{CbAl}_3$  has entirely converted to  $\text{Cb}_2\text{Al}$ , the excellent oxidation resistance characteristics of  $\text{Cb}_3\text{Al}$  are no longer available. Likewise, over a long period of time, as oxygen diffuses into and reacts with the  $\text{Cb}_3\text{Al}$ , it is gradually consumed by conversion into  $\text{Al}_2\text{O}_3$ . Analogous effects take place in coated tantalum and tantalum-base alloys.

When the base metal is columbium or a columbium-base alloy, the monometal trialuminide and di-metal aluminide will be predominantly  $\text{CbAl}_3$  and  $\text{Cb}_2\text{Al}$  respectively. Other elements present in the base metal alloy or in the coating may enter into these compounds. Likewise, when the base metal is tantalum or a tantalum-base alloy, the coating constituents will be  $\text{TaAl}_3$  and  $\text{Ta}_2\text{Al}$ , respectively.

With any of the above variations of the invention, silicon, chromium, titanium or combinations thereof may also be present in the coating. When silicon is present, it has been found to enter into the ductile eutectic formed at the coating-base metal interface along with the silver, aluminum, and columbium or tantalum.

Suitable materials which may be alloyed with columbium comprise tungsten, molybdenum, tantalum, zirconium, and titanium, this list not being a limitation but given only for purposes of illustrating suitable columbium-base alloys. It is, of course, desirable that the percentage of alloying ingredient in either columbium or tantalum base alloys not exceed an amount which would preclude the proper formation of a protective coating on the body.

Columbium alloys containing, about and by weight, tungsten in amounts up to 15 percent, molybdenum from 0 to 5 percent, tantalum from 0 to 33 percent, titanium from 0 to 8 percent, zirconium from 0 to 3 percent, minor amounts of carbon, and the balance essentially all columbium have been found to be suitable for high temperature use. A columbium alloy with which the present invention is particularly useful is known as F-48 and contains nominally, about and by weight, 15 percent tungsten, 5 percent molybdenum, and 1 percent zirconium, balance essentially all columbium. Tantalum alloys containing up to 20 weight percent tungsten, balance essentially all tantalum, are also suitable for use with these coatings at elevated temperatures.

Space age requirements have created an increasing demand for oxidation resistant structural materials. Some columbium-base alloys such as the type shown in Patent 2,973,261, Frank, assigned to the same assignee as the present invention, show excellent strength properties at 2500° F. However, their use has been limited by their low oxidation resistance. Coating requirements include oxidation resistance, ease of application, and prevention of penetration of oxygen and nitrogen, while at the same time the coating must cause minimum reduction in ductility after exposure to air at elevated temperatures. A coating material which appeared to be attractive was aluminum, forming columbium aluminides with the proper heat treatment. Of the columbium aluminides,  $\text{CbAl}_3$  is the most oxidation resistant but unfortunately is also the most brittle.

It is known that when columbium is given an aluminum base coating in an Ag-Al bath the formation of  $\text{CbAl}_3$  is suppressed and the only reaction products formed are  $\text{Cb}_2\text{Al}$  and  $\text{Cb}_3\text{Al}$ . One reason for such action is thought to be that the silver diluting the aluminum causes a decrease in the aluminum activity. This type of coating results in a more ductile structure than former aluminide coatings on columbium, but it must be applied by dipping into a molten metal bath.

According to the present invention, the discovery has been made that a coating of silver prior to the application of an aluminum-base slurry coating resulted in the formation of a coating predominantly of highly oxidation resistant  $\text{CbAl}_3$ . In addition, the silver coating provides at the interface either a silver rich barrier to crack propagation or a silver rich, ductile grain boundary layer or a combination of the two. These effects persist after oxidation testing for over ten hours at 2500° F. in air. The silver in this form was unexpectedly found to inhibit the propagation of cracks through the brittle  $\text{CbAl}_3$  coating matrix and also resulted in an oxidation resistant aluminide coating without causing embrittlement of the base metal. A beneficial effect of the silver plating may be to prevent surface contamination of the base metal by residual oxygen and nitrogen in the argon atmosphere during the fusion treatment and before the outer coatings fuse sufficiently to prevent such contamination.

After a fusion treatment at about 1900° F. for about one hour in a non-oxidizing atmosphere such as argon, a specimen of F-48 columbium alloy that had been silver plated and then slurry coated with an aluminum alloy powder was found to include small entrapped  $\text{Al}_2\text{O}_3$  particles surrounded by a  $\text{CbAl}_3$  matrix. X-ray microemission data indicated that silver and silicon (when an aluminum alloy including silicon is used) are uniformly present throughout the coating, probably in substitutional solid solution be replacement of aluminum atoms in the  $\text{CbAl}_3$  phase. Also the silver was somewhat concentrated at the coating grain boundaries in the region of the coating-base metal interface. After two hours at 2500° F. in air, the columbium-base alloy coated as above was observed to have a first inner portion of substantially all  $\text{Cb}_2\text{Al}$ , an intermediate portion of  $\text{CbAl}_3$  and an outer portion of  $\text{Al}_2\text{O}_3$  with some intermixture of the portions. The coating included progressively more columbium toward the columbium alloy-coating interface.

In the drawings, FIG. 1 is the microstructure at a magnification of 500 $\times$  of coated F-48 alloy which has been silver plated and coated with a slurry of Al-11% Si followed by a slurry of aluminum and then given a one-hour fusion heat treatment at 1900° F. The zones in the coating are identified in the drawing, a continuous phase of  $\text{CbAl}_3$  having dispersed throughout it particles of  $\text{Al}_2\text{O}_3$  remaining from the oxygen in the coating powders. Silver and silicon are diffused throughout the coating, and the interface between the coating and the base metal has etched somewhat differently than the rest of the coating.

FIG. 2 is a 500 $\times$  photomicrograph of the coating of FIG. 1 after a two-hour oxidation treatment at 2500° F. An outer layer of  $\text{Al}_2\text{O}_3$  and an inner layer of  $\text{Cb}_2\text{Al}$  have formed and are indicated in the drawing.

FIG. 3 is an electron micrograph at 16,000 $\times$  of the coated material after the fusion treatment of one hour at 1900° F. in a region near the interface between the coating and the base metal. Particles of the  $\text{Al}_2\text{O}_3$  and a eutectic phase containing silver, silicon and  $\text{CbAl}_3$  are shown.

FIG. 4 is equivalent to FIG. 3 except that it is taken on a sample that has been oxidized in air for two hours at 2500° F. in the region of the interface between the  $\text{CbAl}_3$  and  $\text{Cb}_2\text{Al}$  zones shown in FIG. 2. The eutectic is better defined than in FIG. 3 and appears at the grain boundaries of the  $\text{CbAl}_3$  base.

When even minor amounts of this ductile eutectic preferentially form in a substantial portion of the grain boundary area, it acts as a barrier to propagation of cracks from  $\text{CbAl}_3$  layer into the base metal. Also, the silver diffused in solid solution through the  $\text{CbAl}_3$  (or its equivalent  $\text{TaAl}_3$ ) may also lessen the bulk brittleness of that phase. In any event, coatings of the present invention including silver do not worsen the normally poor ductility and high notch sensitivity of high strength alloys as do similar coatings without the silver content.

The amount of silver required to obtain the advantages of the invention is structurally defined as that amount which will cause silver to come out of solution to form a ductile eutectic at a substantial portion of the grain boundaries with  $\text{CbAl}_3$  or  $\text{TaAl}_3$  as columbium or tantalum diffuses into the coating from the base metal.

In the following examples, percentages are by weight, and mass units are in the avoirdupois system, unless stated otherwise.

The preferred method of applying the coating involves three separate layers and can be called a silver and double-slurry coating treatment. The specimens coated in the following examples were carefully cleaned and degreased panels of F-48 columbium alloy  $1\frac{1}{2}'' \times \frac{1}{2}'' \times 0.020''$  of F-48 columbium alloy with well-rounded edges. First, about 0.001 inch of silver is plated on the base metal. This can be done by vapor plating, electroplating, or any other method of applying a coating of silver. This is followed by an aluminum-11% silicon alloy layer and an aluminum overcoat. Both the aluminum alloy and the aluminum are applied in the form of slurries.

One method of silver plating a base metal by means of an electroplating process would begin with careful surface preparation of the base metal by vapor honing and washing in acetone. This is followed by an acid etch for 20 seconds and subsequent rinsing. The silver plating is done with a silver strike for 45 seconds at 5 volts at room temperature followed by a rinse and then plating in a high speed bath for 5 minutes at 5 volts at 100 to  $120^\circ\text{ F}$ . The silver plated piece is then rinsed and dried. The compositions used in these steps are as follows:

(A) Acid etch bath—

Nitric acid, 20 parts,  
Hydrofluoric acid (48-51%), 20 parts,  
Water, 60 parts.

(B) Silver strike solution—

Silver cyanide 0.25 oz./gal.,  
Copper cyanide 1.50 oz./gal.,  
Sodium cyanide 10.00 oz./gal.

(C) High speed silver plating bath—

Silver cyanide 14-19 oz./gal.,  
Potassium cyanide 15-18 oz./gal.,  
Potassium carbonate 2-10 oz./gal.,  
Potassium hydroxide 0-4 oz./gal.,  
Ammonium thiosulphate (60%), 2 fluid oz./100 gal.

The silver plated base metal is then ready for the double-slurry coating. Both of the slurries are prepared by ball milling the mixtures for a period of 2 to 5 hours. The washed, degreased, and dried silver-plated panel is dipped into a slurry of aluminum-11% silicon (by weight) prealloyed powder using a dip coater at a speed of 8 r.p.m., and the piece to be coated is then removed from the slurry and air dried for 5 minutes. The same process is then repeated with an aluminum powder slurry with the piece subsequently being dried for 8 hours. A typical composition of aluminum-11% silicon slurry follows:

|                                                     | Grams |
|-----------------------------------------------------|-------|
| Al-11% Si powder—325 mesh                           | 100   |
| Xylene                                              | 100   |
| Acryloid (an acrylic resin solution)                | 50    |
| Bentone 34 (dimethyldioctadecyl ammonium bentonite) | 2     |

The powder used in these slurries is prealloyed, meaning that a homogeneous material is formed prior to comminution to powder thereby producing homogeneously al-

loyed powder particles. The aluminum slurry may be composed of:

|                                          | Grams |
|------------------------------------------|-------|
| Reynolds 30LN paste (Al powder—325 mesh) | 250   |
| Xylene                                   | 150   |
| Acetone                                  | 100   |
| Bentone 34                               | 3     |

An Al-11% Si prealloyed powder is preferred for the first slurry coat because of higher fluidity and better wetting of columbium, tantalum and their alloys. However, chromium, titanium or silicon can be used in varying amounts up to about 50 weight percent but preferably less than about 20 weight percent either as a pre-alloy or a mixture with the aluminum metal powder, or alternatively, aluminum metal powder can be used without other metals.

The specimens are now ready for heat treatment. They may be suspended from a support beam in an Inconel boat and heat treated inside in an Inconel retort in an electric muffle furnace. After the muffle had been inserted in the retort it is purged with high purity dry argon. The closed retort is then put into a preheated furnace. After half an hour at  $500^\circ\text{ F}$ . when the volatile components in the slurry are driven off, the temperature is raised to  $1900^\circ\text{ F}$ . At this temperature all three coated layers are liquid. Surface tension will prevent the liquid layers from running off, aluminum oxide covering the surface of the powder particles in the slurries and increasing the viscosity. The panels are held in an argon atmosphere until the liquid constituents react and solidify to form a coherent, oxidation-resistant coating. The retort is then pumped down to less than one micron vacuum and maintained at  $1900^\circ\text{ F}$ . for another half an hour; however, the entire treatment could be carried out in an inert gas atmosphere. Total time of this fusion treatment is about one hour at  $1900^\circ\text{ F}$ .

A preoxidation treatment of exposing a coated and fused article to air at a temperature higher than that of the fusion treatment can be useful for conditioning the coating to provide subsequent protection in air at lower temperatures. This effect results in part from forming a substantial outer layer of  $\text{Al}_2\text{O}_3$  and in part from some of the innermost  $\text{CbAl}$  converting to the more ductile  $\text{Cb}_2\text{Al}$  with silver and perhaps silicon precipitating from solution in the inner layers. This precipitated silver-silicon phase eventually migrates to the grain boundaries and there causes further ductilization. The preoxidation treatment is optional and would be of benefit primarily when the coated articles is to be exposed to an oxidizing atmosphere at relatively low temperatures such as below  $2300^\circ\text{ F}$ . Articles to be exposed to air at higher temperatures will undergo this conditioning in use and a separate preoxidation treatment would be of less value for such articles.

It will readily be seen by those skilled in the art that the preoxidation conditioning treatment will be beneficial even if only one of the two preferred conditions is met. An oxidizing treatment without the higher temperature will produce the  $\text{Al}_2\text{O}_3$  outer layer. A higher temperature than the fusion treatment temperature in a non-oxidizing atmosphere will cause the formation of the  $\text{Cb}_2\text{Al}$  inner layer. However, maximum benefit is obtained from a preoxidation treatment by using a higher temperature than the fusion temperature such as from  $2000^\circ\text{ F}$ . to  $2500^\circ\text{ F}$ ., preferably about  $2300^\circ\text{ F}$ ., and doing the heating in an oxidizing atmosphere such as air.

Standard oxidation tests of the coated panels were carried out in an electric muffle furnace in static air at  $2500^\circ\text{ F}$ . for two hours. Every half hour the samples were taken out of the furnace and inspected for failure. After a ten-hour exposure, the coating showed no sign of edge failure and the bend ductility of the parent or base metal was excellent at room temperature.

Bend tests were performed in a 90° fixture with a 2T radius mandrel on silver-plated and double-slurry coated F-48 columbium alloy panels coated as described above. These tests showed a 90° bend angle at room temperature both after the fusion treatment of one hour at 2500° F. in argon and after subsequent oxidation of two hours at 2500° F. in air.

The coating-base metal system and methods for applying the coatings described in this specification and in the appended claims represent a significant improvement in the art of aluminum-base coatings for columbium and tantalum and alloy systems based on columbium or tantalum. A considerable improvement is found in the ductility properties of bodies coated in accordance with this invention.

What we claim as new and desire to secure by Letters Patent of the United States is:

1. An article of manufacture comprising a body of a base metal selected from the group consisting of columbium, columbium-base alloys, tantalum, and tantalum-base alloys, and a protective coating integral with an exposed surface of said body to protect it against oxidation while not destroying the ductility of the base metal by greatly increasing sensitivity to crack propagation, said coating being bonded together and to said base metal by diffusion and comprising:

a continuous layer of a continuous phase of a monometal trialuminide having a composition in the proportion of one atom at least predominantly of the selected one of the base metals columbium and tantalum to each three atoms of aluminum, said layer containing sufficient amounts of silver in solution so that an excess of the selected one of the base metals columbium and tantalum diffuses into said layer upon exposure to elevated temperatures and an oxidizing atmosphere, a ductile eutectic containing silver, aluminum and the selected one of the base metals columbium and tantalum forms at a substantial portion of the grain boundaries of said monometal trialuminide and acts as a barrier to the propagation of cracks from said layer into said base metal.

2. An article of manufacture according to claim 1 which, upon continued exposure to elevated temperatures and an oxidizing atmosphere, forms a continuous layer

5

of  $\text{Al}_2\text{O}_3$  at its exposed surface and a continuous layer of a di-metal aluminide having a composition in the proportion of two atoms at least predominantly of the selected one of the base metals columbium and tantalum to each atom of aluminum between said monometal trialuminide and said base metal.

10

3. An article of manufacture according to claim 1 in which the coating also contains at least one other metal selected from the group consisting of silicon, chromium and titanium.

15

4. An article of manufacture according to claim 1 in which said ductile eutectic contains silicon in addition to silver, aluminum and the selected one of the base metals columbium and tantalum.

20

5. An article of manufacture according to claim 2 in which the base metal is a columbium-base alloy containing, about and by weight, tungsten in amounts up to 15 percent, molybdenum from 0 to 5 percent, tantalum from 0 to 33 percent, titanium from 0 to 8 percent, zirconium from 0 to 3 percent, minor amounts of carbon, and the balance essentially all columbium, and in which the monometal trialuminide is predominantly  $\text{CbAl}_3$  and the di-metal aluminide is predominantly  $\text{Cb}_2\text{Al}$ .

25

6. An article of manufacture according to claim 5 in which the base metal is a columbium-base alloy consisting essentially of, about and by weight, 15 percent tungsten, 5 percent molybdenum and 1 percent zirconium, balance columbium.

30

7. An article of manufacture according to claim 2 in which the base metal is a tantalum-base alloy containing tungsten in amounts up to about 20 weight percent and the balance essentially all tantalum, and in which the monometal trialuminide is predominantly  $\text{TaAl}_3$  and the di-metal aluminide is predominantly  $\text{Ta}_2\text{Al}$ .

35

40

45

HYLAND BIZOT, Primary Examiner.

#### References Cited by the Examiner

#### UNITED STATES PATENTS

|           |        |         |       |          |
|-----------|--------|---------|-------|----------|
| 3,186,070 | 6/1935 | Oxx     | ----- | 29—198 X |
| 3,205,090 | 9/1965 | Caplow  | ----- | 29—197 X |
| 3,206,289 | 9/1965 | Bradley | ----- | 29—197   |